

# United States Patent [19]

Haruta et al.

[11] Patent Number: 4,544,580

[45] Date of Patent: Oct. 1, 1985

[54] METHOD FOR RECORDING BY WRITING OR PRINTING WITH INK

[75] Inventors: Masahiro Haruta, Funabashi; Takashi Hamamoto, Yokohama; Shigeo Togano, Tokyo, all of Japan

[73] Assignee: Canon Kabushiki Kaisha, Tokyo, Japan

[21] Appl. No.: 640,751

[22] Filed: Aug. 14, 1984

## Related U.S. Application Data

[63] Continuation of Ser. No. 459,987, Jan. 21, 1983, Pat. No. 4,481,244.

## Foreign Application Priority Data

Feb. 3, 1982 [JP] Japan ..... 57-16159  
Feb. 3, 1982 [JP] Japan ..... 57-16160  
Feb. 3, 1982 [JP] Japan ..... 57-16161  
Feb. 3, 1982 [JP] Japan ..... 57-16162  
Feb. 3, 1982 [JP] Japan ..... 57-16163  
Feb. 3, 1982 [JP] Japan ..... 57-16164  
Feb. 3, 1982 [JP] Japan ..... 57-16165  
Feb. 3, 1982 [JP] Japan ..... 57-16166

[51] Int. Cl.<sup>4</sup> ..... B05D 3/00; B05D 5/00

[52] U.S. Cl. ..... 427/261; 346/1.1; 427/288

[58] Field of Search ..... 346/1.1, 135.1; 427/288, 258, 261

## [56] References Cited

### U.S. PATENT DOCUMENTS

3,190,765 6/1965 Yuan ..... 428/315.5  
3,377,191 4/1968 Macnair ..... 428/315.5  
3,922,427 11/1975 Toyoda et al. ..... 428/315.5  
4,346,142 8/1982 Lazear ..... 428/315.7  
4,371,582 2/1983 Sugiyama et al. ..... 428/211  
4,425,405 1/1984 Murakami et al. ..... 428/342  
4,440,827 4/1984 Mujumoto et al. ..... 428/342  
4,442,172 4/1984 Oshima et al. ..... 428/211  
4,481,244 11/1984 Haruta et al. ..... 428/155

### FOREIGN PATENT DOCUMENTS

1007469 10/1965 United Kingdom .

Primary Examiner—William I. Van Balen  
Attorney, Agent, or Firm—Fitzpatrick, Cella, Harper & Scinto

## [57] ABSTRACT

A material used to bear writing or printing, which comprises a substrate and a coating layer formed thereon of a coating material containing a polymer having both hydrophilic segments and hydrophobic segments.

10 Claims, 7 Drawing Figures



FIG. 1



FIG. 2



FIG. 3

 $50\mu\text{m}$ 

FIG. 5

 $50\mu\text{m}$ 

FIG. 4

 $50\mu\text{m}$ 

FIG. 6

 $50\mu\text{m}$ 

FIG. 7

 $50\mu\text{m}$

## METHOD FOR RECORDING BY WRITING OR PRINTING WITH INK

This is a continuation of application Ser. No. 459,987, filed Jan. 21, 1983, now U.S. Pat. No. 4,481,244.

### BACKGROUND OF THE INVENTION

#### 1. Field of the Invention

The present invention relates to materials on which images such as letters and figures are to be written or printed with a recording liquid. Hereinafter, the materials are simply referred to as recording materials.

#### 2. Description of the Prior Art

Recording with a recording liquid or ink has long been made by means of writing tools such as pens, fountain pens, felt pens, etc. Recently, so-called ink-jet recording systems have been developed, where ink is also utilized.

The ink-jet recording system makes a record by forming ink droplets by any of a variety of ink-jetting processes (e.g. electrostatic attractive process, mechanical vibration or displacement process by use of piezoelements, bubbling process where bubbles are generated by impulsive heating, etc.), and leading parts or all of the droplets to adhere onto recording materials such as paper.

For such recording processes using liquid ink, ink is generally required not to blot on recording paper so that the printed letters or figures may not become obscure. The ink is also desired to dry so quickly as to prevent the recording paper from incidental staining with undried ink, and the coloring matter of ink fixed on the paper is desired not to fade out as long as possible.

In particular, the ink-jet recording system should satisfy the following requirements:

- (1) Ink is quickly absorbed into recording paper.
- (2) An ink dot, when overlapping a previously applied ink dot, does not destroy or diffuse the previous ink dot, even in multicolor or full-color recording.
- (3) Ink dots do not diffuse on recording paper and therefore are not enlarged more than needed.
- (4) The shapes of ink dots are close to a perfect circle and the perimeters of ink dots have smooth lines.
- (5) Ink dots have high optical density and distinct perimeter lines.
- (6) Recording paper has a high whiteness and a good contrast of ink dots.
- (7) The color of ink does not vary depending upon the recording paper used.
- (8) Ink droplets scarcely scatter around the dots they form.
- (9) Recording paper exhibits a high dimensional stability without being elongated or wrinkled after recording.

While it has been understood that the satisfying these requirements is also due to characteristics of the recording paper, in practice there has hitherto not been plain paper or specially finished paper that meets the above requirements. For example, the specially finished paper for ink-jet recording disclosed in Japanese Patent Kokai No. 74340/1977, though exhibiting a rapid absorption of ink, is liable to enlarge the diameters of ink dots and to make dim the perimeters of ink dots, and it exhibits a significant change in dimensions after recording.

### SUMMARY OF THE INVENTION

The primary object of this invention is to solve the above problems, unsolved by the prior art, in the present technical field, and, in particular to provide a high performance recording paper which fulfills almost all the above-cited requirements in recording with liquid ink by means of writing tools or ink-jet recording systems.

According to the present invention, there is provided a material used to bear writing or printing which comprises a substrate and a coating layer formed thereon from a coating material containing a polymer having both hydrophilic segments and hydrophobic segments.

### BRIEF DESCRIPTION OF THE DRAWINGS

FIGS. 1 and 2 are illustrations outlining the structure of the recording paper of this invention.

FIGS. 3-7 are traced copies of electron microscopic photographs of coating faces of present recording paper samples.

### DETAILED DESCRIPTION OF PREFERRED EMBODIMENTS

Referring to the drawings and examples, this invention will be illustrated in detail.

In the first place, the construction of this invention is outlined with reference to FIG. 1.

In FIG. 1, numeral 1 represents the liquid-absorption substrate constituted of a porous material, as paper or cloth, or a plastic film or sheet. Numeral 2 represents the coating layer, which receives ink. The coating layer 2 is basically formed from a film-formable coating material containing mainly a polymer having both hydrophilic segments and hydrophobic segments. The coating material may mainly contain both a porous inorganic powder and a polymer having hydrophilic segments along with hydrophobic segments. Further, the coating material may mainly contain a polymer having both hydrophilic segments and hydrophobic and dye-attracting segments. Alternatively, the coating material may mainly contain both a porous inorganic powder and a polymer having hydrophilic segments along with hydrophobic and dye-attracting segments.

Such a polymer can be prepared chiefly from addition-polymerizable vinylic monomers. Hydrophilic segments comprising carboxyl or sulfo groups, or ester groups thereof are introduced in the polymer by using a prescribed amount of an  $\alpha,\beta$ -unsaturated monomer such as acrylic acid, methacrylic acid, crotonic acid, itaconic acid, an itaconic acid monoester, maleic acid, a maleic acid monoester, fumaric acid, a fumaric acid monoester, vinylsulfonic acid, sulfoethyl methacrylate, sulfopropyl methacrylate, or sulfonated vinylnaphthalene.

On the other hand, monomers most suitable for introducing the hydrophobic segments are styrene, styrene derivatives, vinylnaphthalene, vinylnaphthalene derivatives, and esters derived from aliphatic C<sub>8</sub>-C<sub>18</sub> aliphatic alcohols and  $\alpha,\beta$ -ethylenic unsaturated carboxylic acids. In addition to these monomers, for example, the following monomers can be used for the same purpose: acrylonitrile, vinylidene chloride,  $\alpha,\beta$ -ethylenic unsaturated carboxylic acid esters other than the above esters, vinyl acetate, vinyl chloride, acrylamide, methacrylamide, hydroxyethyl methacrylate, hydroxypropyl methacrylate, glycidyl methacrylate, N-methylolacrylamide, N-butoxymethylacrylamide, and the like.

Monomers most suitable for introducing the hydrophobic and dye-attracting segments are, for example, acrylonitrile, vinylidene chloride,  $\alpha, \beta$ -ethylenic unsaturated carboxylic acid esters, vinyl acetate, vinyl chloride, arylamide, methacrylamide, hydroxyethyl methacrylate, hydroxypropyl methacrylate, glycidyl methacrylate, N-methylolacrylamide, N-butoxymethylacrylamide, and the like. In addition to these monomers, there may be used styrene, styrene derivatives, vinyl-naphthalene, vinylnaphthalene derivatives, and esters derived from aliphatic C<sub>8</sub>-C<sub>18</sub> alcohol and  $\alpha, \beta$ -ethylenic unsaturated carboxylic acids.

In this invention, it is necessary to form a salt of the polymer prepared from a combination of the above-cited monomers, for the purpose of making the polymer soluble or colloidally dispersible in the medium of the coating material. Substances combined with the polymer to form the salt include alkali metals such as Na and K; aliphatic amines such as mono-, di-, and tri-methylamines and mono-, di-, and tri-ethylamines; alcohamines such as mono-, di-, and tri-ethanolamines, mono-, di-, tri-propanolamines, methylethanolamine, and dimethylmethylethanolamine; and morpholine and N-methylmorpholine.

A particularly important factor in the present polymer is the proportion of monomer units constituting the hydrophilic segments. When the content of monomer units containing carboxyl group or sulfo group, or ester group thereof, which constitute the hydrophilic segments, exceeds about 40% by weight of the polymer, the so-called sizing effect of the polymer on the substrate 1 is lowered and thereby the ink applied onto the coating layer 2 will blot thereon too much. In addition, the color density of ink fixed is low in this case because the concentration of color-adsorbing sites decreases. On the contrary, the content of hydrophilic monomer units less than 2% by weight lowers the binding force between the coating layer 2 and the substrate 1 making the coating layer 2 readily peelable.

Accordingly, the content of hydrophilic monomer units is preferably about 25 to 40% by weight.

The molecular weight of the polymer is desired to be at least about 2000 since the lower molecular weight deteriorate the film-forming property.

The polymer can be prepared, for instance, in the following way: Essential monomers are mixed in a prescribed ratio and polymerized to a desired molecular weight by a polymerization process such as solution polymerization, emulsion polymerization, or suspension polymerization using a polymerization regulator if necessary. Another acceptable process comprises preparing in the first place a polymer containing acid anhydride, ester, nitrile, or hydroxyl groups, followed by hydrolysis, esterification, sulfate-esterification, or sulfonation of these group, thereby forming hydrophilic groups, such as carboxyl and sulfo groups, in the polymer. The polymer in the form of amine salt may be prepared in any step of the polymer synthesis; for instance, it may be prepared by polymerizing monomer mixtures containing an amine salt of  $\alpha, \beta$ -unsaturated carboxylic acid or adding an amine after polymerization or hydrolysis as mentioned above.

In this invention, one or more of the polymers synthesized as described above are dissolved or dispersed in a solvent to prepare the coating material.

When the polymer is deficient in film-forming property, a binding resin can be incorporated thereto. The binding resin may be water-soluble or organic solvent-

soluble. Water-soluble resins suitable for this purpose include poly(vinyl alcohol), starch, casein, gum arabic, gelatin, polyacrylamide, carboxymethylcellulose, sodium polyacrylate, and sodium alginate. Organic solvent-soluble resins suitable include poly(vinyl butyral), poly(vinyl chloride), poly(vinyl acetate), polyacrylonitrile, poly(methyl methacrylate), poly(vinyl formal), melamine resins, polyamide resins, phenolic resins, polyurethane resins, and alkyd resins.

10 Solvents suitable for the coating material are water and mixtures of water with water-miscible organic solvents.

The water-miscible solvents include alcohols such as methanol, ethanol, n-propanol, isopropanol, n-butanol, 15 sec-butanol, tert-butanol, isobutanol, furfuryl alcohol, and tetrahydrofurfuryl alcohol; ketones or ketoalcohols such as acetone, methyl ethyl ketone, and diacetone alcohol; ethers such as tetrahydrofuran and dioxane; esters such as ethylene carbonate and propylene carbonate; and nitrogen-containing solvents such as N,N-dimethylformamide, N,N-dimethylacetamide, N-methyl-2-pyrrolidone, and diethanolamine.

The porous inorganic particles used jointly with the above-mentioned polymer in the coating material are 25 primarily intended, in this invention, for physical adsorption and capture of the coloring matter (e.g., dye) of the ink applied onto the coating layer 2. Materials effectively used for this purpose are white porous inorganic pigments having an ionic property on the particle surface. Such pigments include natural zeolites, synthetic zeolites (e.g., molecular sieves mfd. by Union Carbide Corp.), diatomaceous earth, finely divided silica (average particle size up to 1 $\mu$ ), powdered silica (average particle size up to 20 $\mu$ ), and synthetic mica 30 (represented by the formula M.Mg<sub>2.5</sub>(Si<sub>4</sub>O<sub>10</sub>)<sub>2</sub>F<sub>2</sub>, wherein M is hydrogen or metal atom).

In this invention, one or more kinds of these inorganic particles (generally particle sizes of microns to 40 hundreds of microns) are dispersed in the coating solvent along with one or more of the above-mentioned polymers dissolved or dispersed.

The coating layer 2 can be formed by applying the coating material onto the substrate 1 in a known coating way (e.g., roll coating, rod bar coating, spray coating, or the like) so as to give a dry coating weight generally of ca. 1-10 g/m<sup>2</sup>, preferably of ca. 2-5 g/m<sup>2</sup> from a more practical aspect. The coating material is then dried as soon as possible.

When ink is applied onto the coating layer 2, the 50 coloring matter (e.g., dye) of the ink is selectively adsorbed and captured therein by forming ionic bonds, hydrogen bonds, or the like with the polymer and physical bonds with the porous inorganic particles.

Furthermore, regulation of the composition of the 55 coating material and the film-forming conditions, in particular the drying conditions after coating, gives a coating layer such as the following: As shown in FIG. 2-2L, which is a ca. 50-fold magnified view of part 21 of the coating layer 2 surface, numerous fine scale-like lamellae are two-dimensionally densely arranged, said lamellae being separated from one another by micro-cracks 4 running at random (mostly as deep as reaching the surface of the substrate 1). The dimensions or geometry of each scale-like lamellae 3 are not particularly 60 limited but approximately 10 $\mu$  × 10 $\mu$  to hundreds  $\mu$  × hundreds  $\mu$  in general. The width of each micro-crack 4 is also not particularly limited but usually several  $\mu$ . The dimensions or geometry of the scale-like

lamellae 3 and the widths of the micro-cracks 4 can be varied at will within the above respective ranges by regulating or controlling the composition of the coating material and the film-forming conditions, in particular the drying conditions after coating.

When ink is applied onto the coating layer 2, the coloring matter (e.g., dye) of the ink is selectively adsorbed and captured in the scale-like lamellae 3 by forming ionic bonds or hydrogen bonds, or the like with the polymer and physical bonds with the porous inorganic particles, while the solvent of the ink passes through the micro-cracks 4 and is quickly absorbed into the substrate 1. Thus, the coloring matter of ink, on recording, is mostly captured by the upper-most zone of recording paper, so that excellent coloration of the applied ink is obtainable. On the other hand, the solvent of the ink rapidly moves through the micro-cracks to the underlying substrate, so that the ink on the paper surface is rapidly brought into an apparently dry state.

In addition, the scale-like lamellae 3 are particularly effective in preventing the applied ink dots from being enlarged more than needs or from being dim at the perimeters, thus giving ink dots of high optical density. This is caused by the intensive adsorption of the coloring matter of ink in the scale-like lamellae 3. The power of this adsorption principally depends upon chemical properties of the polymer (e.g., the ionic character) and physical properties of the inorganic particles (e.g., the voids).

It is undesirable that the surface area occupied by the scale-like lamellae 3 of the whole surface area of recording paper is excessively small, in other words, the surface area occupied by the micro-cracks 4 is extremely large. In such a case, the efficiency of capturing the coloring matter is lowered, resulting in a poor coloration or low optical density of ink dots; the amount of ink migrating to the substrate 1 increases, giving rise to a so-called back penetration phenomenon of ink; and the shapes of ink dots become worse. Accordingly, the conditions leading to such a state of the coating layer should be avoided.

This invention will be illustrated in more detail with reference to Examples and the effect of this invention will be demonstrated.

Samples of the polymer, a main component of the coating layer in this invention, used in the Examples were prepared as shown in the following Preparation Examples or were the commercial ones shown below: In the Examples and Preparation Examples, "parts" means parts by weight.

50

#### PREPARATION EXAMPLE 1

A mixture of water (50 parts), isopropanol (30 parts), sodium dodecylbenzenesulfonate (0.5 part), and ammonium persulfate (0.5 part) was heated to 60° C. in a four-necked separable flask equipped with a stirrer and a dropping funnel. A mixture of styrene (5 parts), acrylic acid (9 parts), and butyl acrylate (5 parts) was added dropwise thereto from the dropping funnel over 60 minutes. After completion of the addition, the temperature was raised to 80° C. and the polymerization was conducted for 2 hours with stirring. The molecular weight of the polymer obtained was about 50,000.

#### PREPARATION EXAMPLE 2

Methyl methacrylate (8 parts), styrene (5 parts), itaconic acid (15 parts), benzoyl peroxide (1 part), lauryl mercaptan (1 part), diacetone alcohol (50 parts), and

ethylene glycol (20 parts) were charged in the same flask as used in Preparation Example 1. The polymerization was conducted for 6 hours under a stream of nitrogen. The molecular weight of the polymer obtained was about 30,000.

In the following Preparation Examples, polymers were obtained from the following respective feeds in the same manner as in Preparation Example 2.

#### PREPARATION EXAMPLE 3

|                                           |          |
|-------------------------------------------|----------|
| Styrene                                   | 10 parts |
| Acrylonitrile                             | 5 parts  |
| Methacrylic acid                          | 10 parts |
| Hydroxyethyl methacrylate                 | 5 parts  |
| Azobisisobutyronitrile                    | 1 parts  |
| Ethylene glycol monomethyl ether          | 19 parts |
| Butanol                                   | 50 parts |
| (Molecular weight of polymer: ca. 15,000) |          |

#### PREPARATION EXAMPLE 4

|                                           |          |
|-------------------------------------------|----------|
| Vinylnaphthalene                          | 10 parts |
| N,N-Dimethyl-methacrylamide               | 5 parts  |
| Maleic anhydride                          | 10 parts |
| Methyl ethyl ketone peroxide              | 1 parts  |
| Isopropanol                               | 60 parts |
| Diethanolamine                            | 14 parts |
| (Molecular weight of polymer: ca. 20,000) |          |

#### PREPARATION EXAMPLE 5

|                                           |          |
|-------------------------------------------|----------|
| Styrene                                   | 10 parts |
| Maleic anhydride                          | 10 parts |
| Diethanolamine                            | 2 parts  |
| Azobisisobutyronitrile                    | 1 parts  |
| Ethyl acrylate                            | 5 parts  |
| Ethyl-carbitol                            | 23 parts |
| Diethylene glycol monomethyl ether        | 50 parts |
| (Molecular weight of polymer: ca. 30,000) |          |

#### PREPARATION EXAMPLE 6

|                                          |          |
|------------------------------------------|----------|
| Styrene                                  | 5 parts  |
| Itaconic acid monoethyl ester            | 5 parts  |
| Methacrylic acid                         | 10 parts |
| 2-Ethylhexyl methacrylate                | 10 parts |
| Benzoyl peroxide                         | 1 parts  |
| Thiomalic acid                           | 1 parts  |
| n-Propanol                               | 48 parts |
| Ethylene glycol                          | 20 parts |
| (Molecular weight of polymer: ca. 8,000) |          |

#### COMMERCIAL POLYMERS

- Sodium naphthalenesulfonate-formalin condensation polymer:



(n = 3-10)

Trade name: Demol N (Kao-Altal Inc.)

- b. Diisobutylene-maleic acid copolymer Trade name: 15 Demol EP (Kao-Atlas Inc.)  
 c. Sodium polyacrylate Trade name: Nopcosant R (San-Nopco Co., Ltd.)  
 d. Ammonium polyacrylate Trade name: Nopcosant RFA (San-Nopco Co., Ltd.)  
 e. Sodium polymethacrylate Trade name: Primal 850 20 (Rohm & Haas Co.)  
 f. Styrene-maleic acid monoester ammonium salt copolymer



(m = 6-8)

Trade name: SMA Resin 1440H (Alco Chem. Co.)

- g. Polyethylene glycol Trade name: Macrogol 1500 35 (Nippon Yushi Co., Ltd.)  
 h. Polyethylene glycol-polypropylene glycol block copolymer Trade name: Uniroope 40DP-50B (Nippon Yushi Co., Ltd.)

In the following Examples, a coating material (usually in slurry form) for forming the coating layer was applied to coat one side of base paper so as to give a dry coating weight of approximately 4 g/m<sup>2</sup>.

Ink-jet recording tests in the following Examples, recording characteristics of recording paper samples 45 were determined as follows:

The optical density of ink dot of the characteristics was determined by using a microdensitometer (PDM-5, mfd. by Konishiroku Photographic Ind. Co., Ltd.) with a 30μ×30μ slit at a recorded sample speed of 10μ/sec. 50 in the x-axial direction and a chart speed of 1 mm/sec (speed ratio of sample to chart: 1/100).

The diameter of ink dots were measured by use of a microscope.

The fixation time for ink of the characteristics is the 55 time passed from the application of an ink droplet onto a sample paper until the ink comes not to adhere to the surface or a rubber press roll placed at a definite position apart in the sample-forwarding direction from the ink-jetting head used; said time was determined by 60 varying the sample speed, in other words, varying the time passed from the application of ink dot until the ink dot contacts with the rubber roll. The diameter of ink-jetting orifice of the ink-jetting head used was 50μ.

#### EXAMPLE 1

The following compositions were thoroughly stirring and mixed severally to prepared five kinds of slurry:

| Composition A |                                                    |           |
|---------------|----------------------------------------------------|-----------|
|               | Polymer obtained in Preparation                    | 100 parts |
| 5             | Example 1                                          |           |
|               | Water                                              | 150 parts |
| Composition B |                                                    |           |
|               | Polymer obtained in Preparation                    | 100 parts |
| 10            | Example 2                                          |           |
|               | Water                                              | 100 parts |
|               | Ethanol                                            | 50 parts  |
| Composition C |                                                    |           |
|               | Polymer obtained in Preparation                    | 80 parts  |
| 15            | Example 6                                          |           |
|               | Poly(vinyl alcohol)                                | 20 parts  |
|               | Water                                              | 100 parts |
| Composition D |                                                    |           |
|               | Demol N (a commercial polymer cited above)         | 70 parts  |
| 20            | Gelatin                                            | 20 parts  |
|               | Water                                              | 100 parts |
|               | Methanol                                           | 20 parts  |
| Composition E |                                                    |           |
|               | SMA Resin 1440H (a correrical polymer cited above) | 50 parts  |
| 25            | Sodium alginate                                    | 50 parts  |
|               | Water                                              | 150 parts |

The slurries were separately applied onto base paper (basis weight 60 g/m<sup>2</sup>) and forcibly dried in the usual 30 way to prepare Samples I-V of recording paper. Results of the ink-jet recording tests of these samples are summarized in Table 1. The ink used was of the following composition and properties:

#### Ink composition:

|                               |          |
|-------------------------------|----------|
| Water Black 187L (Orient Co.) | 10 parts |
| Diethylene glycol             | 30 parts |
| Water                         | 60 parts |

#### Ink properties:

|                  |                                                                                                                   |
|------------------|-------------------------------------------------------------------------------------------------------------------|
| Viscosity:       | 3.8 cps., as measured with a rotation viscometer (E-type, mfd. by Tokyo Keiki Co., Ltd.).                         |
| Surface tension: | 52.4 dyne/cm, as measured with a plate-suspension type of surface tension meter (mfd. by Kyowa Kagaku Co., Ltd.). |

TABLE 1

| Sam-<br>ple<br>No. | Compo-<br>nition of<br>slurry | Number of<br>ink dots<br>superposed<br>(note 1) | Recording characteristics           |                                    |                                 |                              |
|--------------------|-------------------------------|-------------------------------------------------|-------------------------------------|------------------------------------|---------------------------------|------------------------------|
|                    |                               |                                                 | Optical<br>density<br>of ink<br>dot | Di-<br>ameter<br>of ink<br>dot (μ) | Fixa-<br>tion<br>time<br>(sec.) | Image<br>quality<br>(note 2) |
| I                  | A                             | 1                                               | 0.85                                | 110                                | 0.9                             |                              |
|                    |                               | 3                                               | 1.05                                | 165                                | 2.5                             | ○                            |
|                    |                               | 4                                               | 1.21                                | 180                                | 3.6                             |                              |
| II                 | B                             | 1                                               | 0.88                                | 100                                | 0.7                             |                              |
|                    |                               | 3                                               | 1.10                                | 130                                | 2.0                             | ○                            |
|                    |                               | 4                                               | 1.25                                | 155                                | 2.6                             |                              |
| III                | C                             | 1                                               | 0.90                                | 105                                | 0.8                             |                              |
|                    |                               | 3                                               | 1.12                                | 130                                | 2.4                             | ○                            |
|                    |                               | 4                                               | 1.28                                | 160                                | 2.9                             |                              |
| IV                 | D                             | 1                                               | 0.87                                | 125                                | 0.9                             |                              |
|                    |                               | 3                                               | 1.10                                | 140                                | 2.6                             | ○                            |
|                    |                               | 4                                               | 1.26                                | 185                                | 3.8                             |                              |
| V                  | E                             | 1                                               | 0.91                                | 110                                | 0.8                             |                              |
|                    |                               | 3                                               | 1.15                                | 135                                | 2.3                             | ○                            |

TABLE 1-continued

| Sam-<br>ple<br>No. | Compo-<br>sition of<br>slurry | Recording characteristics                       |                                     |                                          |                                 |                              |
|--------------------|-------------------------------|-------------------------------------------------|-------------------------------------|------------------------------------------|---------------------------------|------------------------------|
|                    |                               | Number of<br>ink dots<br>superposed<br>(note 1) | Optical<br>density<br>of ink<br>dot | Dia-<br>meter<br>of ink<br>dot ( $\mu$ ) | Fix-<br>ation<br>time<br>(sec.) | Image<br>quality<br>(note 2) |
|                    |                               | 4                                               | 1.30                                | 155                                      | 2.8                             |                              |

Note 1:  
Number of ink droplets successively applied to the same point on the recording paper.  
Note 2:  
Evaluation criteria  
◎ excellent  
○ good

## EXAMPLE 2

A slurry was prepared by thorough stirring and mixing the polymer (100 parts) obtained in Preparation Example 3, water (110 parts), and ethanol (50 parts). The slurry was applied onto base paper (basis weight 65 g/m<sup>2</sup>) and dried under the same conditions as in Example 1 to prepare a recording paper sample.

The ink-jet recording tests of this sample gave nearly the same results as in the case of Sample V of Example 1.

## EXAMPLES 3 AND 4

Sample II of recording paper prepared in Example 1 was tested for said ink-jet recording characteristics using inks of the following compositions: The results were as shown in Table 2.

## COMPOSITION OF INK

## EXAMPLE 3

|                      |          |
|----------------------|----------|
| C.I. Direct Black 19 | 5 parts  |
| Ethylene glycol      | 70 parts |
| Water                | 25 parts |

## EXAMPLE 4

|                    |          |
|--------------------|----------|
| Spilon Black GMH   | 10 parts |
| Triethylene glycol | 40 parts |
| monomethyl ether   |          |
| Ethanol            | 50 parts |

TABLE 2

| Example<br>No. | Number of<br>ink dots<br>superposed<br>(note 1) | Recording characteristics           |                                  |                                 |                              |
|----------------|-------------------------------------------------|-------------------------------------|----------------------------------|---------------------------------|------------------------------|
|                |                                                 | Optical<br>density<br>of ink<br>dot | Diameter of<br>ink dot ( $\mu$ ) | Fix-<br>ation<br>time<br>(sec.) | Image<br>quality<br>(note 2) |
| 3              | 1                                               | 0.80                                | 80                               | 0.8                             |                              |
|                | 2                                               | 1.01                                | 90                               | 1.6                             |                              |
|                | 3                                               | 1.21                                | 95                               | 1.9                             | ◎                            |
|                | 4                                               | 1.32                                | 110                              | 2.2                             |                              |
| 4              | 5                                               | 1.38                                | 125                              | 3.5                             |                              |
|                | 1                                               | 0.82                                | 80                               | 0.8                             |                              |
|                | 2                                               | 1.10                                | 88                               | 1.5                             |                              |
|                | 3                                               | 1.21                                | 105                              | 2.0                             | ◎                            |
|                | 4                                               | 1.25                                | 123                              | 2.2                             |                              |
|                | 5                                               | 1.36                                | 136                              | 3.6                             |                              |

Notes 1 and 2 are the same with those of Table 1.

## EXAMPLE 5

Full-color ink-jet recording tests of Sample III of Example 1 by use of cyanin, magenta, yellow, and black inks gave nearly the same results as in the case of Sam-

ple III of Example 1 with respect to fixation time, optical density of ink dot, and diameter of ink dot. Thus, full-color photographs could be duplicated wherein all the colors were extremely clear and exhibited good reproducibility.

## EXAMPLE 6

Writing tests by use of a commercial fountain pen were made on the Samples of recording paper prepared in Example 1. All the samples exhibited quick absorption of ink without ink running thereon, thus very beautiful letters being written.

## EXAMPLE 7

A slurry was prepared by thorough stirring and mixing the polymer (100 parts) obtained in Preparation Example 1 and water (150 parts). The slurry was applied onto base paper (basis weight 60 g/m<sup>2</sup>) and dried under the following five different conditions to prepare Samples VI-X of recording paper.

| Drying conditions: |                                                  |
|--------------------|--------------------------------------------------|
| 25                 | Sample VI                                        |
|                    | Natural drying by leaving the specimen standing. |
| 30                 | Sample VII                                       |
|                    | In a 60° C. oven for 2 hours.                    |
|                    | Sample VIII                                      |
|                    | In a stream of 90° C. hot air for 30 minutes.    |
|                    | Sample IX                                        |
|                    | In a stream of 110° C. hot air for 1 minute.     |
|                    | Sample X                                         |
|                    | In a stream of 180° C. hot air for 2 seconds.    |

Electron microscopic photographs (magnification factor 200) of coating faces of the samples are shown in FIGS. 3-7.

The samples thus obtained were tested for said ink-jet recording characteristics using the same ink as used in Example 1. The results are shown in Table 3.

TABLE 3

| Sam-<br>ple<br>No. | Magnified<br>appearance<br>of coating<br>face | Number<br>of ink<br>dots<br>super-<br>posed<br>(note 1) | Recording characteristics           |                                          |                                 |                              |
|--------------------|-----------------------------------------------|---------------------------------------------------------|-------------------------------------|------------------------------------------|---------------------------------|------------------------------|
|                    |                                               |                                                         | Optical<br>density<br>of ink<br>dot | Dia-<br>meter<br>of ink<br>dot ( $\mu$ ) | Fix-<br>ation<br>time<br>(sec.) | Image<br>quality<br>(note 2) |
| VI                 | FIG. 3                                        | 1                                                       | 0.82                                | 150                                      | 1.0                             | X                            |
|                    |                                               | 2                                                       | 0.91                                | 170                                      | 1.8                             |                              |
|                    |                                               | 3                                                       | 1.00                                | 200                                      | 3.2                             |                              |
|                    |                                               | 4                                                       | 1.21                                | 260                                      | 6.7                             |                              |
| VII                | FIG. 4                                        | 5                                                       | 1.27                                | 310                                      | 10.0                            |                              |
|                    |                                               | 1                                                       | 0.85                                | 130                                      | 0.9                             | △                            |
|                    |                                               | 2                                                       | 0.93                                | 165                                      | 1.5                             |                              |
|                    |                                               | 3                                                       | 1.07                                | 200                                      | 2.7                             |                              |
| VIII               | FIG. 5                                        | 4                                                       | 1.17                                | 220                                      | 4.6                             |                              |
|                    |                                               | 5                                                       | 1.28                                | 270                                      | 8.2                             |                              |
|                    |                                               | 1                                                       | 0.88                                | 90                                       | 0.6                             | △                            |
|                    |                                               | 2                                                       | 1.07                                | 115                                      | 0.8                             |                              |
| IX                 | FIG. 6                                        | 3                                                       | 1.18                                | 126                                      | 1.5                             |                              |
|                    |                                               | 4                                                       | 1.30                                | 135                                      | 2.1                             |                              |
|                    |                                               | 5                                                       | 1.36                                | 150                                      | 3.1                             |                              |
|                    |                                               | 1                                                       | 0.90                                | 95                                       | 0.5                             |                              |
| X                  | FIG. 7                                        | 2                                                       | 1.06                                | 110                                      | 0.7                             |                              |
|                    |                                               | 3                                                       | 1.23                                | 115                                      | 1.0                             | ○                            |
|                    |                                               | 4                                                       | 1.32                                | 123                                      | 1.5                             |                              |
|                    |                                               | 5                                                       | 1.37                                | 135                                      | 2.2                             |                              |
| 65                 | X                                             | 1                                                       | 0.90                                | 90                                       | 0.3                             |                              |
|                    |                                               | 2                                                       | 1.09                                | 105                                      | 0.6                             |                              |
|                    |                                               | 3                                                       | 1.20                                | 113                                      | 1.0                             | ◎                            |
|                    |                                               | 4                                                       | 1.28                                | 120                                      | 1.3                             |                              |

TABLE 3-continued

| Sam-<br>ple<br>No. | Magnified<br>appearance<br>of coating<br>face | Number<br>of ink<br>dots<br>(note 1) | Recording characteristics           |                                          |                                 |                              |
|--------------------|-----------------------------------------------|--------------------------------------|-------------------------------------|------------------------------------------|---------------------------------|------------------------------|
|                    |                                               |                                      | Optical<br>density<br>of ink<br>dot | Di-<br>ameter<br>of ink<br>dot ( $\mu$ ) | Fix-<br>ation<br>time<br>(sec.) | Image<br>quality<br>(note 2) |
|                    |                                               | 5                                    | 1.36                                | 125                                      | 1.7                             |                              |

Note 1: the same with that of Table 1.

Note 2: Evaluation criteria:

◎ excellent,  
○ good,  
△ fair,  
X poor

## EXAMPLE 8

A slurry was prepared by thorough stirring and mixing the polymer (100 parts) obtained in Preparation Example 3, water (110 parts), and ethanol (50 parts). The slurry was applied onto base paper (basis weight 65 g/m<sup>2</sup>) and dried in a stream of 180°C. hot air for a few seconds to prepare a sample of recording paper.

Electron microscopic photographs of the coating surface exhibited nearly the appearance as shown by FIG. 7.

The ink-jet recording tests of this sample gave nearly the same results as of Sample X of Example 7.

## EXAMPLE 9

A slurry was prepared by thorough stirring and mixing the polymer (80 parts) obtained in Preparation Example 6, a poly(vinyl alcohol) (20 parts), and water (150 parts). Then, a sample of recording paper was prepared and tested in the same manner as in Example 8, giving nearly equal results.

## EXAMPLES 10 AND 11

Sample X prepared in Example 7 was tested for ink-jet recording characteristics using the same inks as used in Examples 3 and 4, respectively. The results are shown in Table 4.

TABLE 4

| Ex-<br>am-<br>No. | Ink used                           | Recording Characteristics                       |                                     |                                          |                                 |                              |
|-------------------|------------------------------------|-------------------------------------------------|-------------------------------------|------------------------------------------|---------------------------------|------------------------------|
|                   |                                    | Number of<br>ink dots<br>superposed<br>(note 1) | Optical<br>density<br>of ink<br>dot | Di-<br>ameter<br>of ink<br>dot ( $\mu$ ) | Fix-<br>ation<br>time<br>(sec.) | Image<br>quality<br>(note 2) |
| 10                | Same as<br>used in<br>Example<br>3 | 1                                               | 0.80                                | 80                                       | 0.3                             |                              |
|                   |                                    | 2                                               | 1.01                                | 90                                       | 0.6                             |                              |
|                   |                                    | 3                                               | 1.21                                | 95                                       | 0.9                             | ◎                            |
|                   |                                    | 4                                               | 1.32                                | 110                                      | 1.2                             |                              |
|                   |                                    | 5                                               | 1.38                                | 125                                      | 1.5                             |                              |
| 11                | Same as<br>used in<br>Example<br>4 | 1                                               | 0.82                                | 80                                       | 0.2                             |                              |
|                   |                                    | 2                                               | 1.10                                | 88                                       | 0.5                             |                              |
|                   |                                    | 3                                               | 1.21                                | 105                                      | 0.9                             | ◎                            |
|                   |                                    | 4                                               | 1.25                                | 123                                      | 1.2                             |                              |
|                   |                                    | 5                                               | 1.36                                | 136                                      | 1.6                             |                              |

Note 1 and 2 are the same with those of Table 1.

## EXAMPLE 12

Full-color ink-jet recording tests of Sample X of Example 7 by use of cyanin, magenta, yellow, and black inks gave nearly the same results as in the case of Sample X of Example 7 with respect to fixation time, optical density of ink dots, and diameter of ink dot. Thus, full-color photographs could be duplicated wherein all the colors were very clear and were good in reproducibility.

EXAMPLE 13

Writing tests by use of a commercial fountain pen were made on the recording paper prepared in Example 8. The recording paper exhibited quick absorption of ink without ink running thereon, thus very beautiful letters being written.

## EXAMPLE 14

The following Compositions were thoroughly mixed and ground severally to prepare five kinds of slurry.

| Composition F                                      |           |
|----------------------------------------------------|-----------|
| Polymer obtained in Preparation Example 1          | 100 parts |
| Silica powder                                      | 50 parts  |
| Water                                              | 150 parts |
| Composition G                                      |           |
| Polymer obtained in Preparation Example 2          | 100 parts |
| Silica powder                                      | 100 parts |
| Water                                              | 100 parts |
| Ethanol                                            | 50 parts  |
| Composition H                                      |           |
| Polymer obtained in Preparation Example 6          | 80 parts  |
| Diatomaceous earth                                 | 80 parts  |
| Poly(vinyl alcohol)                                | 20 parts  |
| Water                                              | 100 parts |
| Composition J                                      |           |
| Demol N (a commercial polymer cited above)         | 70 parts  |
| Synthetic zeolite                                  | 80 parts  |
| Gelatin                                            | 20 parts  |
| Water                                              | 100 parts |
| Methanol                                           | 20 parts  |
| Composition K                                      |           |
| SMA Resin 1440H (a commercial polymer cited above) | 50 parts  |
| Diatomaceous earth                                 | 70 parts  |
| Sodium alginate                                    | 50 parts  |
| Water                                              | 150 parts |

Each slurry was applied onto base paper (basis weight 60 g/m<sup>2</sup>) and forcibly dried to prepare Samples XI-XV of recording paper.

The samples were tested for the ink-jet recording characteristics using the same ink as used in Example 1. The results are shown in Table 5.

TABLE 5

| Sam-<br>ple<br>No. | Compo-<br>sition of<br>slurry | Number of<br>ink dots<br>superposed<br>(note 1) | Recording characteristics           |                                          |                                 |                              |
|--------------------|-------------------------------|-------------------------------------------------|-------------------------------------|------------------------------------------|---------------------------------|------------------------------|
|                    |                               |                                                 | Optical<br>density<br>of ink<br>dot | Di-<br>ameter<br>of ink<br>dot ( $\mu$ ) | Fix-<br>ation<br>time<br>(sec.) | Image<br>quality<br>(note 2) |
| XI                 | F                             | 1                                               | 0.87                                | 85                                       | 0.6                             |                              |
|                    |                               | 3                                               | 1.07                                | 100                                      | 1.5                             | ◎                            |
|                    |                               | 4                                               | 1.23                                | 130                                      | 2.7                             |                              |
|                    |                               | 5                                               | 1.27                                | 125                                      | 2.6                             |                              |
| XII                | G                             | 1                                               | 0.90                                | 80                                       | 0.6                             |                              |
|                    |                               | 3                                               | 1.12                                | 105                                      | 1.8                             | ◎                            |
|                    |                               | 4                                               | 1.27                                | 125                                      | 2.6                             |                              |
|                    |                               | 5                                               | 1.30                                | 130                                      | 2.9                             |                              |
| XIII               | H                             | 1                                               | 0.92                                | 83                                       | 0.8                             |                              |
|                    |                               | 3                                               | 1.14                                | 102                                      | 2.0                             | ◎                            |
|                    |                               | 4                                               | 1.30                                | 130                                      | 2.9                             |                              |
|                    |                               | 5                                               | 1.12                                | 110                                      | 2.6                             | ○                            |
| XIV                | J                             | 1                                               | 0.89                                | 95                                       | 0.9                             |                              |
|                    |                               | 3                                               | 1.12                                | 110                                      | 2.6                             | ○                            |
|                    |                               | 4                                               | 1.28                                | 135                                      | 3.8                             |                              |
|                    |                               | 5                                               | 1.32                                | 120                                      | 2.6                             |                              |
| XV                 | K                             | 1                                               | 0.92                                | 83                                       | 0.7                             |                              |
|                    |                               | 3                                               | 1.17                                | 105                                      | 1.8                             | ◎                            |
|                    |                               | 4                                               | 1.32                                | 120                                      | 2.6                             |                              |

Notes 1 and 2 are the same with those of Table 1.

## EXAMPLE 15

A slurry prepared by thorough stirring and mixing the polymer (100 parts) obtained in Preparation Example 3, a silica powder (70 parts), water (110 parts), and ethanol (50 parts) was applied onto base paper (basis weight 65 g/m<sup>2</sup>) and dried under the same conditions as in Example 14 to prepare a sample of recording paper. The ink-jet recording tests of this sample gave nearly the same results as in case of Sample XV of Example 14. 10

## EXAMPLES 16 AND 17

Sample XI of recording paper prepared in Example 14 was tested for the ink-jet recording characteristics using the same inks as used in Examples 3 and 4, respectively. The results are shown in Table 6. 15

TABLE 6

| Ex-<br>am-<br>ple<br>No. | Ink used                           | Recording characteristics                       |                                     |                                    |                                 |                              |
|--------------------------|------------------------------------|-------------------------------------------------|-------------------------------------|------------------------------------|---------------------------------|------------------------------|
|                          |                                    | Number of<br>ink dots<br>superposed<br>(note 1) | Optical<br>density<br>of ink<br>dot | Di-<br>ameter<br>of ink<br>dot (μ) | Fix-<br>ation<br>time<br>(sec.) | Image<br>quality<br>(note 2) |
| 16                       | Same as<br>used in<br>Example<br>3 | 1                                               | 0.80                                | 80                                 | 0.8                             |                              |
|                          |                                    | 2                                               | 1.01                                | 90                                 | 1.6                             |                              |
|                          |                                    | 3                                               | 1.21                                | 95                                 | 1.9                             | ◎                            |
|                          |                                    | 4                                               | 1.32                                | 110                                | 2.2                             |                              |
|                          |                                    | 5                                               | 1.38                                | 125                                | 3.5                             |                              |
| 17                       | Same as<br>used in<br>Example<br>4 | 1                                               | 0.82                                | 80                                 | 0.7                             |                              |
|                          |                                    | 2                                               | 1.10                                | 88                                 | 1.5                             |                              |
|                          |                                    | 3                                               | 1.21                                | 105                                | 2.0                             | ◎                            |
|                          |                                    | 4                                               | 1.25                                | 123                                | 2.4                             |                              |
|                          |                                    | 5                                               | 1.36                                | 136                                | 3.6                             |                              |

Notes 1 and 2 are the same with those of Table 1.

## EXAMPLE 18

Full-color ink-jet recording tests of Sample XIII of Example 14 by use of cyanin, magenta, yellow, and black inks gave nearly the same results as in the case of Sample XIII of Example 14 with respect to the fixation time, optical density of ink dot, and diameter of ink dot. Thus, full-color photographs could be duplicated wherein all the colors were very clear and were good in reproducibility. 35

## EXAMPLE 19

Writing tests by use of a commercial fountain pen were made on the samples of recording paper prepared in Example 14. All the samples exhibited quick absorption of ink, without ink running thereon, thus very beautiful letters being written. 45

## EXAMPLE 20

A slurry was prepared by thorough stirring and mixing the polymer (30 parts) obtained in Preparation Example 1, a silica powder (50 parts), and water (150 parts). The slurry was applied onto base paper (basis weight 60 g/m<sup>2</sup>) and dried under the following five different conditions to prepare Samples XVI-XX of recording paper: 50

| Drying Conditions: |                                                  |
|--------------------|--------------------------------------------------|
| Sample XVI         | Natural drying by leaving the specimen standing. |
| Sample XVII        | In a 60° C. oven for 2 hours.                    |
| Sample XVIII       | In a stream of 90° C. hot air for 30 minutes.    |
| Sample XIX         | In a stream of 110° C. hot air for 1 minute.     |
| Sample XX          | In a stream of 180° C. hot                       |

-continued

## Drying Conditions:

air for 2 seconds.

5

Electron microscopic photographs (magnification factor 200) of coating faces of the samples were not much different from those shown in FIGS. 3-7.

The samples were tested for the ink-jet recording characteristics using the same ink as used in Example 1. The results are shown in Table 7.

TABLE 7

| Sample<br>No. | Mag-<br>nified<br>appear-<br>ance of<br>coating<br>face | Number<br>of ink<br>dots<br>super-<br>posed<br>(note 1) | Recording characteristics           |                                    |                                 |                              |
|---------------|---------------------------------------------------------|---------------------------------------------------------|-------------------------------------|------------------------------------|---------------------------------|------------------------------|
|               |                                                         |                                                         | Optical<br>density<br>of ink<br>dot | Di-<br>ameter<br>of ink<br>dot (μ) | Fix-<br>ation<br>time<br>(sec.) | Image<br>quality<br>(note 2) |
| XVI           | As<br>shown in<br>FIG. 3                                | 1                                                       | 0.86                                | 150                                | 1.0                             | X                            |
|               |                                                         | 2                                                       | 0.95                                | 160                                | 1.5                             |                              |
|               |                                                         | 3                                                       | 1.03                                | 200                                | 2.6                             |                              |
|               |                                                         | 4                                                       | 1.28                                | 260                                | 6.3                             |                              |
|               |                                                         | 5                                                       | 1.32                                | 310                                | 10.0                            |                              |
| XVII          | As<br>shown in<br>FIG. 4                                | 1                                                       | 0.88                                | 140                                | 0.9                             | △                            |
|               |                                                         | 2                                                       | 0.96                                | 155                                | 1.7                             |                              |
|               |                                                         | 3                                                       | 1.12                                | 180                                | 2.8                             |                              |
|               |                                                         | 4                                                       | 1.24                                | 220                                | 5.5                             |                              |
| XVIII         | As<br>shown in<br>FIG. 5                                | 1                                                       | 0.95                                | 110                                | 0.5                             | △                            |
|               |                                                         | 2                                                       | 1.13                                | 115                                | 0.6                             |                              |
|               |                                                         | 3                                                       | 1.26                                | 120                                | 1.3                             |                              |
|               |                                                         | 4                                                       | 1.33                                | 135                                | 2.1                             |                              |
|               |                                                         | 5                                                       | 1.41                                | 150                                | 3.0                             |                              |
| XIX           | As<br>shown in<br>FIG. 6                                | 1                                                       | 0.96                                | 95                                 | 0.4                             |                              |
|               |                                                         | 2                                                       | 1.15                                | 110                                | 0.6                             |                              |
|               |                                                         | 3                                                       | 1.28                                | 115                                | 1.0                             | ○                            |
|               |                                                         | 4                                                       | 1.36                                | 120                                | 1.5                             |                              |
|               |                                                         | 5                                                       | 1.43                                | 130                                | 2.0                             |                              |
| XX            | As<br>shown in<br>FIG. 7                                | 1                                                       | 0.95                                | 90                                 | 0.3                             |                              |
|               |                                                         | 2                                                       | 1.16                                | 105                                | 0.5                             |                              |
|               |                                                         | 3                                                       | 1.28                                | 115                                | 1.0                             | ◎                            |
|               |                                                         | 4                                                       | 1.39                                | 120                                | 1.2                             |                              |
|               |                                                         | 5                                                       | 1.45                                | 125                                | 1.6                             |                              |

40 Notes 1 and 2 are the same with those of Table 3.

## EXAMPLE 21

A slurry prepared by thorough stirring and mixing the polymer (50 parts) obtained in Preparation Example 3, diatomaceous earth (70 parts), and water (100 parts) was applied onto base paper (basis weight 65 g/m<sup>2</sup>) and dried in a stream of 180° C. hot air for a few seconds to prepare a sample of recording paper. 35

Electron microscopic photographs of the coating surface exhibited nearly the same appearance as shown by FIG. 7. 50

The ink-jet recording tests of this sample gave nearly the same results as in the case of Sample XX of Example 20. 55

## EXAMPLE 22

A slurry was prepared by thorough stirring and mixing the polymer (80 parts) obtained in Preparation Example 6, a synthetic zeolite (130 parts), a poly(vinyl alcohol)(20 parts), water(250 parts) and methanol (100 parts). Then, a sample of recording paper was prepared and tested in the same manner as in Example 21, giving nearly equal results. 60

## EXAMPLES 23 AND 24

Sample XX prepared in Example 20 was tested for the ink-jet recording characteristics using the same inks

65

as used in Examples 3 and 4. The results are shown in Table 8.

TABLE 8

| Ex-<br>am-<br>ple<br>No. | Ink used                           | Number of<br>ink dots<br>superposed<br>(note 1) | Recording characteristics           |                                          |                                 |                              |
|--------------------------|------------------------------------|-------------------------------------------------|-------------------------------------|------------------------------------------|---------------------------------|------------------------------|
|                          |                                    |                                                 | Optical<br>density<br>of ink<br>dot | Di-<br>ameter<br>of ink<br>dot ( $\mu$ ) | Fix-<br>ation<br>time<br>(sec.) | Image<br>quality<br>(note 2) |
| 23                       | Same as<br>used in<br>Example<br>3 | 1                                               | 0.82                                | 80                                       | 0.3                             | ◎                            |
|                          |                                    | 2                                               | 1.03                                | 90                                       | 0.6                             |                              |
|                          |                                    | 3                                               | 1.21                                | 98                                       | 1.0                             |                              |
|                          |                                    | 4                                               | 1.35                                | 110                                      | 1.3                             |                              |
|                          |                                    | 5                                               | 1.41                                | 125                                      | 1.7                             |                              |
| 24                       | Same as<br>used in<br>Example<br>4 | 1                                               | 0.85                                | 85                                       | 0.2                             | ◎                            |
|                          |                                    | 2                                               | 1.10                                | 92                                       | 0.6                             |                              |
|                          |                                    | 3                                               | 1.23                                | 110                                      | 0.9                             |                              |
|                          |                                    | 4                                               | 1.29                                | 128                                      | 1.2                             |                              |
|                          |                                    | 5                                               | 1.38                                | 140                                      | 1.6                             |                              |

Notes 1 and 2 are the same with those of Table 1.

## EXAMPLE 25

Full-color ink-jet recording tests of Sample XX of Example 20 by use of cyanin, magenta, yellow, and black inks gave nearly the same results as in the case of Sample XX of Example 20 with respect to the fixation time, optical density of ink dots, and diameter of ink dot. Thus, full-color photographs could be duplicated wherein all the colors were very clear and were good in reproducibility.

## EXAMPLE 26

Writing tests by use of a commercial fountain pen were made on the sample of recording paper prepared in Example 21. The sample exhibited quick absorption of ink without ink running thereon, thus very beautiful letters being written.

## EXAMPLE 27

The following compositions were thoroughly stirring and mixed severally to prepare five kinds of slurry:

| <u>Composition L</u>                      |           |
|-------------------------------------------|-----------|
| Polymer obtained in Preparation Example 6 | 100 parts |
| Water                                     | 150 parts |
| <u>Composition M</u>                      |           |
| Polymer obtained in Preparation Example 4 | 100 parts |
| Water                                     | 100 parts |
| Ethanol                                   | 50 parts  |
| <u>Composition N</u>                      |           |
| Polymer obtained in Preparation Example 6 | 80 parts  |
| Poly(vinyl alcohol)                       | 20 parts  |
| Water                                     | 100 parts |
| <u>Composition P</u>                      |           |
| Polymer obtained in Preparation Example 3 | 70 parts  |
| Gelatin                                   | 20 parts  |
| Water                                     | 100 parts |
| Methanol                                  | 20 parts  |
| <u>Composition Q</u>                      |           |
| Polymer obtained in Preparation Example 4 | 50 parts  |
| Sodium alginate                           | 50 parts  |
| Water                                     | 150 parts |

The slurries were separately applied onto base paper (basis weight 60 g/m<sup>2</sup>) and forcibly dried in the usual way to prepare Samples XXI-XXV of recording paper.

These samples were tested for the ink-jet recording characteristics using the same ink as used in Example 1. The results are summarized in Table 9.

TABLE 9

| 5  | Sample<br>No. | Compo-<br>sition<br>of<br>slurry | Number<br>of ink<br>dots<br>super-<br>posed<br>(note 1) | Recording characteristics           |                                          |                                 |                              |
|----|---------------|----------------------------------|---------------------------------------------------------|-------------------------------------|------------------------------------------|---------------------------------|------------------------------|
|    |               |                                  |                                                         | Optical<br>density<br>of ink<br>dot | Di-<br>ameter<br>of ink<br>dot ( $\mu$ ) | Fix-<br>ation<br>time<br>(sec.) | Image<br>quality<br>(note 2) |
| 10 | XXI           | L                                | 1                                                       | 0.87                                | 95                                       | 0.7                             | ◎                            |
|    |               |                                  | 3                                                       | 1.06                                | 135                                      | 2.0                             |                              |
|    |               |                                  | 4                                                       | 1.23                                | 150                                      | 2.8                             |                              |
|    | XXII          | M                                | 1                                                       | 0.90                                | 100                                      | 0.8                             |                              |
|    |               |                                  | 3                                                       | 1.10                                | 140                                      | 2.3                             |                              |
| 15 | XXIII         | N                                | 1                                                       | 0.92                                | 90                                       | 0.6                             | ◎                            |
|    |               |                                  | 3                                                       | 1.15                                | 130                                      | 1.8                             |                              |
|    |               |                                  | 4                                                       | 1.33                                | 145                                      | 2.5                             |                              |
|    | XXIV          | P                                | 1                                                       | 0.88                                | 110                                      | 0.9                             |                              |
|    |               |                                  | 3                                                       | 1.12                                | 155                                      | 2.7                             |                              |
| 20 | XXV           | Q                                | 1                                                       | 0.90                                | 105                                      | 0.9                             | ○                            |
|    |               |                                  | 3                                                       | 1.13                                | 152                                      | 2.8                             |                              |
|    |               |                                  | 4                                                       | 1.30                                | 180                                      | 3.8                             |                              |

Notes 1 and 2 are the same with those of Table 1.

## EXAMPLES 28 AND 29

Sample XXIII of recording paper prepared in Example 27 was tested for the ink-jet recording characteristics using the same inks as used in Examples 3 and 4, respectively. The results are shown in Table 10.

TABLE 10

| Ex-<br>am-<br>ple<br>No. | Ink used                           | Number of<br>ink dots<br>superposed<br>(note 1) | Recording characteristics           |                                          |                                 |                              |
|--------------------------|------------------------------------|-------------------------------------------------|-------------------------------------|------------------------------------------|---------------------------------|------------------------------|
|                          |                                    |                                                 | Optical<br>density<br>of ink<br>dot | Di-<br>ameter<br>of ink<br>dot ( $\mu$ ) | Fix-<br>ation<br>time<br>(sec.) | Image<br>quality<br>(note 2) |
| 28                       | Same as<br>used in<br>Example<br>3 | 1                                               | 0.80                                | 80                                       | 0.8                             | ◎                            |
|                          |                                    | 2                                               | 1.01                                | 90                                       | 1.6                             |                              |
|                          |                                    | 3                                               | 1.21                                | 95                                       | 1.8                             |                              |
|                          |                                    | 4                                               | 1.32                                | 110                                      | 2.0                             |                              |
|                          |                                    | 5                                               | 1.38                                | 125                                      | 3.5                             |                              |
| 29                       | Same as<br>used in<br>Example<br>4 | 1                                               | 0.82                                | 80                                       | 0.7                             | ◎                            |
|                          |                                    | 2                                               | 1.10                                | 88                                       | 1.5                             |                              |
|                          |                                    | 3                                               | 1.21                                | 105                                      | 1.9                             |                              |
|                          |                                    | 4                                               | 1.25                                | 123                                      | 2.2                             |                              |
|                          |                                    | 5                                               | 1.36                                | 136                                      | 3.6                             |                              |

Notes 1 and 2 are the same with those of Table 1.

## EXAMPLE 30

Full-color ink-jet recording tests of Sample XXIII of Example 27 by use of cyanin, magenta, yellow, and black inks gave nearly the same results as in the case of Sample XXIII of Example 27 with respect to fixation time, optical density of ink dot, and diameter of ink dot. Thus, a full-color photograph could be duplicated wherein all the colors were extremely clear and were good in reproducibility.

## EXAMPLE 31

Writing tests by use of a commercial fountain pen were made on the samples of recording paper prepared in Example 27. All the samples exhibited quick absorption of ink without ink running thereon, thus very beautiful letters being written.

## EXAMPLE 32

A slurry was prepared by thorough stirring and mixing the polymer (100 parts) obtained in Preparation

Example 6 and water (150 parts). The slurry was applied onto base paper (basis weight 60 g/m<sup>2</sup>) and dried under the following five different conditions to prepare Samples XXVI-XXX of recording paper.

| Dry conditions: |                                                  |
|-----------------|--------------------------------------------------|
| Sample XXVI     | Natural drying by leaving the specimen standing. |
| Sample XXVII    | In a 60° C. oven for 2 hours.                    |
| Sample XXVIII   | In a stream of 90° C. hot air for 30 minutes.    |
| Sample XXIX     | In a stream of 110° C. hot air for 1 minute.     |
| Sample XXX      | In a stream of 180° C. hot air for 2 seconds.    |

Electron microscopic photographs (magnification factor 200) of coating faces of the samples were not much different from those shown in FIGS. 3-7.

The samples thus obtained were subjected to the ink-jet recording tests with the same ink as used in Example 1. The results are shown in Table 11.

TABLE 11

| Sample No. | Mag-<br>nified<br>appear-<br>ance of<br>coating<br>face | Number<br>of ink<br>dots<br>super-<br>posed<br>(note 1) | Recording characteristics           |                                    |                                 |                                 |
|------------|---------------------------------------------------------|---------------------------------------------------------|-------------------------------------|------------------------------------|---------------------------------|---------------------------------|
|            |                                                         |                                                         | Optical<br>density<br>of ink<br>dot | Di-<br>ameter<br>of ink<br>dot (μ) | Fix-<br>ation<br>time<br>(sec.) | Image<br>quality<br>(note<br>2) |
| XXVI       | As shown in FIG. 3                                      | 1                                                       | 0.82                                | 150                                | 1.0                             | X                               |
|            |                                                         | 2                                                       | 0.91                                | 170                                | 1.8                             |                                 |
|            |                                                         | 3                                                       | 1.00                                | 200                                | 3.2                             |                                 |
|            |                                                         | 4                                                       | 1.21                                | 260                                | 6.7                             |                                 |
|            |                                                         | 5                                                       | 1.27                                | 310                                | 10.0                            |                                 |
| XXVII      | As shown in FIG. 4                                      | 1                                                       | 0.85                                | 130                                | 0.9                             | Δ                               |
|            |                                                         | 2                                                       | 0.93                                | 165                                | 1.5                             |                                 |
|            |                                                         | 3                                                       | 1.07                                | 200                                | 2.7                             |                                 |
|            |                                                         | 4                                                       | 1.17                                | 220                                | 4.6                             |                                 |
|            |                                                         | 5                                                       | 1.28                                | 270                                | 8.2                             |                                 |
| XXVIII     | As shown in FIG. 5                                      | 1                                                       | 0.88                                | 90                                 | 0.6                             | Δ                               |
|            |                                                         | 2                                                       | 1.07                                | 115                                | 0.8                             |                                 |
|            |                                                         | 3                                                       | 1.18                                | 126                                | 1.5                             |                                 |
|            |                                                         | 4                                                       | 1.30                                | 135                                | 2.1                             |                                 |
|            |                                                         | 5                                                       | 1.36                                | 150                                | 3.1                             |                                 |
| XXIX       | As shown in FIG. 6                                      | 1                                                       | 0.90                                | 95                                 | 0.5                             |                                 |
|            |                                                         | 2                                                       | 1.06                                | 110                                | 0.7                             |                                 |
|            |                                                         | 3                                                       | 1.23                                | 115                                | 1.0                             | ○                               |
|            |                                                         | 4                                                       | 1.32                                | 123                                | 1.5                             |                                 |
|            |                                                         | 5                                                       | 1.37                                | 135                                | 2.2                             |                                 |
| XXX        | As shown in FIG. 7                                      | 1                                                       | 0.90                                | 90                                 | 0.3                             |                                 |
|            |                                                         | 2                                                       | 1.09                                | 105                                | 0.6                             | ○                               |
|            |                                                         | 3                                                       | 1.20                                | 113                                | 1.0                             | ○                               |
|            |                                                         | 4                                                       | 1.28                                | 120                                | 1.3                             |                                 |
|            |                                                         | 5                                                       | 1.36                                | 125                                | 1.7                             |                                 |

Notes 1 and 2 are the same with those of Table 3.

## EXAMPLE 33

A slurry prepared by thorough stirring and mixing the polymer (100 parts) obtained in Preparation Example 3, water (110 parts), and ethanol (50 parts) was applied onto base paper (basis weight 65 g/m<sup>2</sup>) and dried in a stream of 180° C. hot air for a few seconds to prepare a sample of recording paper.

Electron microscopic photographs of the coating surface exhibited nearly the same appearance as shown by FIG. 7.

Ink-jet recording tests of this sample gave nearly the same results as of Sample XXX of Example 32.

## EXAMPLE 34

A slurry was prepared by thorough stirring and mixing the polymer (80 parts) obtained in Preparation Ex-

ample 4, a poly(vinyl alcohol) (20 parts), and water (150 parts). Then, a sample of recording paper was prepared and tested in the same manner as in Example 33, giving nearly equal results.

5

## EXAMPLES 35 AND 36

The sample prepared in Example 33 was tested for the ink-jet recording characteristic using the same inks as used in Examples 3 and 4, respectively. The results are shown in Table 12.

| Ex-<br>am-<br>ple<br>No. | Ink used                  | Recording characteristics                       |                                     |                                    |                              |
|--------------------------|---------------------------|-------------------------------------------------|-------------------------------------|------------------------------------|------------------------------|
|                          |                           | Number of<br>ink dots<br>superposed<br>(note 1) | Optical<br>density<br>of ink<br>dot | Di-<br>ameter<br>of ink<br>dot (μ) | Image<br>quality<br>(note 2) |
| 35                       | Same as used in Example 3 | 1                                               | 0.80                                | 80                                 | 0.3                          |
|                          | 2                         | 1.01                                            | 90                                  | 0.6                                |                              |
|                          | 3                         | 1.21                                            | 95                                  | 0.9                                | ○                            |
|                          | 4                         | 1.32                                            | 110                                 | 1.2                                |                              |
|                          | 5                         | 1.38                                            | 125                                 | 1.5                                |                              |
| 36                       | Same as used in Example 4 | 1                                               | 0.82                                | 80                                 | 0.2                          |
|                          | 2                         | 1.10                                            | 88                                  | 0.5                                |                              |
|                          | 3                         | 1.21                                            | 105                                 | 0.9                                | ○                            |
|                          | 4                         | 1.25                                            | 123                                 | 1.2                                |                              |
|                          | 5                         | 1.36                                            | 136                                 | 1.6                                |                              |

Notes 1 and 2 are the same with those of Table 1.

## EXAMPLE 37

Full-color ink-jet recording tests of the sample of Example 34 by use of cyanin, magenta, yellow, and black inks gave nearly the same results as in the case of Sample XXX of Example 32 with respect to fixation time, optical density of ink dot, and diameter of ink dot. Thus, fullcolor photographs could be duplicated wherein all the colors were very clear and were good in reproducibility.

## EXAMPLE 38

Writing tests by use of a commercial fountain pen were made on the recording paper prepared in Example 33. The recording paper exhibited quick absorption of ink without ink running thereon, thus very beautiful letters being written.

## EXAMPLE 39

The following compositions were thoroughly mixed and ground severally to prepare five kinds of slurry.

| Composition R                             |           |
|-------------------------------------------|-----------|
| Polymer obtained in Preparation Example 6 | 100 parts |
| Silica powder                             | 50 parts  |
| Water                                     | 150 parts |
| Composition S                             |           |
| Polymer obtained in Preparation Example 4 | 100 parts |
| Silica powder                             | 100 parts |
| Water                                     | 100 parts |
| Ethanol                                   | 50 parts  |
| Composition T                             |           |
| Polymer obtained in Preparation Example 6 | 80 parts  |
| Diatomaceous earth                        | 80 parts  |
| Poly(vinyl alcohol)                       | 20 parts  |
| Water                                     | 100 parts |
| Composition U                             |           |
| Polymer obtained in Preparation Example 3 | 70 parts  |
| Synthetic zeolite                         | 80 parts  |

-continued

|                                 |           |
|---------------------------------|-----------|
| Gelatin                         | 20 parts  |
| Water                           | 100 parts |
| Methanol                        | 20 parts  |
| <u>Composition V</u>            |           |
| Polymer obtained in Preparation | 50 parts  |
| <u>Example 4</u>                |           |
| Diatomaceous earth              | 70 parts  |
| Sodium alginate                 | 50 parts  |
| Water                           | 150 parts |

Each slurry was applied onto base paper (basis weight 60 g/m<sup>2</sup>) and forcibly dried in the usual way to prepare Samples XXXI-XXXV of recording paper.

These samples were tested for the ink-jet recording characteristics using the same ink as used in Example 1. The results are shown in Table 13.

TABLE 13

| Sample No. | Com-<br>posi-<br>tion of<br>slurry | Number<br>of ink<br>dots<br>super-<br>posed<br>(note 1) | Recording characteristics           |                                    |                                 |                              |
|------------|------------------------------------|---------------------------------------------------------|-------------------------------------|------------------------------------|---------------------------------|------------------------------|
|            |                                    |                                                         | Optical<br>density<br>of ink<br>dot | Di-<br>ameter<br>of ink<br>dot (μ) | Fix-<br>ation<br>time<br>(sec.) | Image<br>quality<br>(note 2) |
| XXXI       | R                                  | 1                                                       | 0.88                                | 83                                 | 0.5                             |                              |
|            |                                    | 3                                                       | 1.07                                | 93                                 | 1.8                             | ◎                            |
|            |                                    | 4                                                       | 1.24                                | 118                                | 2.6                             |                              |
| XXXII      | S                                  | 1                                                       | 0.92                                | 80                                 | 0.6                             |                              |
|            |                                    | 3                                                       | 1.11                                | 98                                 | 2.1                             | ◎                            |
|            |                                    | 4                                                       | 1.33                                | 112                                | 2.8                             |                              |
| XXXIII     | T                                  | 1                                                       | 0.93                                | 88                                 | 0.4                             |                              |
|            |                                    | 3                                                       | 1.16                                | 100                                | 1.6                             | ◎                            |
|            |                                    | 4                                                       | 1.34                                | 113                                | 2.3                             |                              |
| XXXIV      | U                                  | 1                                                       | 0.89                                | 92                                 | 0.7                             |                              |
|            |                                    | 3                                                       | 1.13                                | 112                                | 2.5                             | ○                            |
|            |                                    | 4                                                       | 1.28                                | 120                                | 3.4                             |                              |
| XXXV       | V                                  | 1                                                       | 0.90                                | 82                                 | 0.7                             |                              |
|            |                                    | 3                                                       | 1.13                                | 96                                 | 2.3                             | ○                            |
|            |                                    | 4                                                       | 1.30                                | 115                                | 3.2                             |                              |

Notes 1 and 2 are the same with those of Table 1.

## EXAMPLES 40 AND 41

Sample XXXIII of recording paper prepared in Example 39 was tested for the ink-jet recording characteristics using the same inks as used in Examples 3 and 4. The results are shown in Table 14.

TABLE 14

| Ex-<br>am-<br>ple<br>No. | Ink used                           | Number of<br>ink dots<br>superposed<br>(note 1) | Recording characteristics           |                                    |                                 |                              |
|--------------------------|------------------------------------|-------------------------------------------------|-------------------------------------|------------------------------------|---------------------------------|------------------------------|
|                          |                                    |                                                 | Optical<br>density<br>of ink<br>dot | Di-<br>ameter<br>of ink<br>dot (μ) | Fix-<br>ation<br>time<br>(sec.) | Image<br>quality<br>(note 2) |
| 40                       | Same as<br>used in<br>Example<br>3 | 1                                               | 0.80                                | 80                                 | 0.8                             |                              |
|                          |                                    | 2                                               | 1.01                                | 90                                 | 1.6                             |                              |
|                          |                                    | 3                                               | 1.21                                | 95                                 | 1.8                             | ◎                            |
|                          |                                    | 4                                               | 1.32                                | 110                                | 2.2                             |                              |
|                          |                                    | 5                                               | 1.38                                | 125                                | 3.5                             |                              |
| 41                       | Same as<br>used in<br>Example<br>3 | 1                                               | 0.82                                | 80                                 | 0.7                             |                              |
|                          |                                    | 2                                               | 1.10                                | 88                                 | 1.5                             |                              |
|                          |                                    | 3                                               | 1.21                                | 105                                | 1.9                             | ◎                            |
|                          |                                    | 4                                               | 1.25                                | 123                                | 2.2                             |                              |
|                          |                                    | 5                                               | 1.36                                | 136                                | 3.6                             |                              |

Notes 1 and 2 are the same with those of Table 1.

## EXAMPLE 42

Full-color ink-jet recording tests of Sample XXXIII of Example 39 by use of cyanin, magenta, yellow, and black inks gave nearly the same results as in the case of Sample XXXIII of Example 39 with respect to the fixation time, optical density of ink dot, and diameter of ink dot. Thus, full-color photographs could be dupli-

cated wherein all the colors were very clear and were good in reproducibility.

## EXAMPLE 43

Writing tests by use of a commercial fountain pen were made on the samples of recording paper prepared in Example 37. All the samples exhibited quick absorption of ink without ink running thereon, thus very beautiful letters being written.

## EXAMPLE 44

A slurry was prepared by thorough stirring and mixing the polymer (30 parts) obtained in Preparation Example 6, a silica powder (50 parts), and water (150 parts) was applied onto base paper (basis weight 60 g/m<sup>2</sup>) and dried under the following five different conditions to prepare Samples XXXVI-XXXX of recording paper:

| Drying Conditions: |                                                  |
|--------------------|--------------------------------------------------|
| Sample XXXVI       | Natural drying by leaving the specimen standing. |
| Sample XXXVII      | In a 60° C. oven for 2 hours.                    |
| Sample XXXVIII     | In a stream of 90° C. hot air for 30 minutes.    |
| Sample XXXIX       | In a stream of 110° C. hot air for 1 minute.     |
| Sample XXXX        | In a stream of 180° C. hot air for 2 seconds.    |

Electron microscopic photographs (magnification factor 200) of coating faces of the samples were not much different from those shown in FIGS. 3-7.

The samples were tested for the ink-jet recording characteristics using the same ink as used in Example 1. The results are shown in Table 15.

TABLE 15

| Sample<br>No. | Mag-<br>nified<br>appear-<br>ance of<br>coating<br>face | Number<br>of ink<br>dots<br>super-<br>posed<br>(note 1) | Recording characteristics           |                                    |                                 |   | Im-<br>age<br>qual-<br>ity<br>(note<br>2) |
|---------------|---------------------------------------------------------|---------------------------------------------------------|-------------------------------------|------------------------------------|---------------------------------|---|-------------------------------------------|
|               |                                                         |                                                         | Optical<br>density<br>of ink<br>dot | Di-<br>ameter<br>of ink<br>dot (μ) | Fix-<br>ation<br>time<br>(sec.) |   |                                           |
| XXXVI         | As<br>shown<br>in FIG. 3                                | 1                                                       | 0.86                                | 150                                | 1.0                             | X |                                           |
|               |                                                         | 2                                                       | 0.95                                | 160                                | 1.5                             |   |                                           |
|               |                                                         | 3                                                       | 1.03                                | 200                                | 2.6                             |   |                                           |
|               |                                                         | 4                                                       | 1.28                                | 260                                | 6.3                             |   |                                           |
|               |                                                         | 5                                                       | 1.32                                | 310                                | 10.0                            |   |                                           |
| XXXVII        | As<br>shown<br>in FIG. 4                                | 1                                                       | 0.88                                | 140                                | 0.9                             | Δ |                                           |
|               |                                                         | 2                                                       | 0.96                                | 155                                | 1.3                             |   |                                           |
|               |                                                         | 3                                                       | 1.12                                | 180                                | 2.2                             |   |                                           |
|               |                                                         | 4                                                       | 1.24                                | 220                                | 5.5                             |   |                                           |
|               |                                                         | 5                                                       | 1.33                                | 270                                | 8.2                             |   |                                           |
| XXXVIII       | As<br>shown<br>in FIG. 5                                | 1                                                       | 0.95                                | 110                                | 0.5                             | Δ |                                           |
|               |                                                         | 2                                                       | 1.13                                | 115                                | 0.6                             |   |                                           |
|               |                                                         | 3                                                       | 1.26                                | 120                                | 1.3                             |   |                                           |
|               |                                                         | 4                                                       | 1.33                                | 135                                | 2.1                             |   |                                           |
|               |                                                         | 5                                                       | 1.41                                | 150                                | 3.0                             |   |                                           |
| XXXIX         | As<br>shown<br>in FIG. 6                                | 1                                                       | 0.96                                | 95                                 | 0.4                             |   |                                           |
|               |                                                         | 2                                                       | 1.15                                | 110                                | 0.6                             |   |                                           |
|               |                                                         | 3                                                       | 1.28                                | 115                                | 1.0                             | ○ |                                           |
|               |                                                         | 4                                                       | 1.36                                | 120                                | 1.5                             |   |                                           |
|               |                                                         | 5                                                       | 1.43                                | 130                                | 2.0                             |   |                                           |
| XXXX          | As<br>shown<br>in FIG. 7                                | 1                                                       | 0.95                                | 90                                 | 0.3                             |   |                                           |
|               |                                                         | 2                                                       | 1.16                                | 105                                | 0.5                             |   |                                           |
|               |                                                         | 3                                                       | 1.28                                | 115                                | 1.0                             | ◎ |                                           |
|               |                                                         | 4                                                       | 1.39                                | 120                                | 1.2                             |   |                                           |
|               |                                                         | 5                                                       | 1.45                                | 125                                | 1.6                             |   |                                           |

Notes 1 and 2 are the same with those of Table 3.

## EXAMPLE 45

A slurry prepared by thorough stirring and mixing the polymer (50 parts) obtained in Preparation Example 3, diatomaceous earth (70 parts), and ethanol (50 parts) was applied onto base paper (65 g/m<sup>2</sup>) and dried in a stream of 180° C. hot air for a few seconds to prepare a sample of recording paper.

Electron microscopic photographs of the coating surface exhibited nearly the same appearance as shown by FIG. 7.

The ink-jet recording tests of this sample gave nearly the same results as in the case of Sample XXXX of Example 44.

## EXAMPLE 46

A slurry was prepared by thorough mixing the polymer (80 parts) obtained in Preparation Example 4, a synthetic zeolite (130 parts), a poly(vinyl alcohol)(20 parts), water (250 parts) and methanol (100 parts). Then, a sample of recording paper was prepared and tested in the same manner as in Example 45, giving nearly equal results.

## EXAMPLES 47 AND 48

The sample prepared in Example 45 was tested for the ink-jet recording characteristics using the same inks as used in Examples 3 and 4, respectively. The results are shown in Table 16.

TABLE 16

| Ex-<br>am-<br>ple<br>No. | Ink used                           | Number of<br>ink dots<br>superposed<br>(note 1) | Recording characteristics           |                                    |                                 |                              |
|--------------------------|------------------------------------|-------------------------------------------------|-------------------------------------|------------------------------------|---------------------------------|------------------------------|
|                          |                                    |                                                 | Optical<br>density<br>of ink<br>dot | Di-<br>ameter<br>of ink<br>dot (μ) | Fix-<br>ation<br>time<br>(sec.) | Image<br>quality<br>(note 2) |
| 47                       | Same as<br>used in<br>Example<br>3 | 1                                               | 0.82                                | 80                                 | 0.3                             |                              |
|                          |                                    | 2                                               | 1.03                                | 90                                 | 0.6                             |                              |
|                          |                                    | 3                                               | 1.21                                | 98                                 | 1.0                             | ◎                            |
|                          |                                    | 4                                               | 1.35                                | 110                                | 1.3                             |                              |
|                          |                                    | 5                                               | 1.41                                | 125                                | 1.7                             |                              |
| 48                       | Same as<br>used in<br>Example<br>4 | 1                                               | 0.85                                | 85                                 | 0.2                             |                              |
|                          |                                    | 2                                               | 1.10                                | 92                                 | 0.6                             |                              |
|                          |                                    | 3                                               | 1.23                                | 110                                | 0.9                             | ◎                            |
|                          |                                    | 4                                               | 1.29                                | 128                                | 1.2                             |                              |
|                          |                                    | 5                                               | 1.38                                | 140                                | 1.6                             |                              |

Notes 1 and 2 are the same with those of Table 1.

## EXAMPLE 49

Full-color ink-jet recording tests of the sample of Example 46 by use of cyanin, magenta, yellow, and black inks gave nearly the same results as in the case of Sample XXXX of Example 44 with respect to the fixation time, optical density of ink dot, and diameter of ink dot. Thus, full-color photographs could be duplicated wherein all the colors were very clear and were good in reproducibility.

## EXAMPLE 50

Writing tests by use of a commercial fountain pen were made on the sample of recording paper prepared in Example 45. The sample exhibited quick absorption

of ink without ink running thereon, thus very beautiful letters being written.

As described hereinbefore, this invention provides recording paper excellent in recording performance characteristics and best suited for multicolor ink-jet recording, particularly in the following respects:

The recording liquid (ink) applied onto the recording paper is quickly absorbed thereinto, that is to say, the coloring matter of ink is quickly fixed to the upper zone of the paper and the solvent of ink is also quickly absorbed into the underlying zone of the paper. Even when ink droplets different in color are applied successively in short periods of time to the same point of the paper face, no significant running or blotting of ink occurs thereon, in other words, the spread of ink dots can be inhibited within such an extent as not to impair the clearness of image, and thus good coloration is obtainable.

We claim:

1. A method for recording by writing or printing with ink, the method comprising the steps of:

providing a material to bear the writing or printing, said material including a substrate of a recording paper suitable for ink recording and a coating layer formed thereon of a coating material containing a polymer having both hydrophilic segments and hydrophobic segments; and depositing ink on said material.

2. The method according to claim 1, wherein said coating material also includes porous inorganic powder.

3. The method according to claim 1, wherein said coating layer includes a plurality of micro-cracks having the capacity of passing liquid therethrough.

4. The method according to claim 1, wherein said substrate is formed of a porous material.

5. The method according to claim 1, wherein said hydrophobic segments of the polymer have an affinity for coloring matter.

6. The method according to claim 1, wherein said coating layer is formed of a resin coating material capable of forming a film.

7. The method according to claim 6, wherein said resin coating material contains a surfactant.

8. The method according to claim 1, wherein said coating layer is formed by coating the substrate with a coating material to give a dry coating weight of 1 to 10 g/m<sup>2</sup>.

9. The method according to claim 1, wherein ink is deposited on the material by ink-jet recording.

10. A method for preparing color images by ink-jet recording, the method comprising the steps of:

forming droplets, each being one of a plurality of colors of recording liquids, including black recording liquid; and

depositing said droplets on a material including a substrate of a recording paper suitable for ink-jet recording and a coating layer formed thereon of a coating material containing a polymer having both hydrophilic segments and hydrophobic segments.

\* \* \* \* \*

UNITED STATES PATENT AND TRADEMARK OFFICE  
CERTIFICATE OF CORRECTION

PATENT NO. : 4,544,580  
DATED : October 1, 1985  
INVENTOR(S) : MASAHIRO HARUTA, ET AL.

Page 1 of 2

It is certified that error appears in the above-identified patent and that said Letters Patent is hereby corrected as shown below:

Column 1, line 59, change "that the satisfying" to --that satisfying--.

Column 2, line 5, change "particular to" to --particular, to--.

Column 3, line 44, change "deteriorate" to --deteriorates--.

Column 5, line 22, change "needs" to --needed--.

Column 6, line 7, change "folloiwng" to --following--;

line 19, change "1 parts" to --1 part--;  
line 31, change "1 parts" to --1 part--;  
line 44, change "1 parts" to --1 part--;  
line 58, change "1 parts" to --1 part--;

and

line 59, change "1 parts" to --1 part--.

Column 7, line 13, change "Kao-Altal" to --Kao-Atlas--;

line 58, change "surface or" to --surface of--;

line 67, change "stirring" to --stirred--; and

line 68, change "to prepared" to --to prepare--.

Column 8, line 23, change "correcial" to --commercial--.

UNITED STATES PATENT AND TRADEMARK OFFICE  
CERTIFICATE OF CORRECTION

PATENT NO. : 4,544,580  
DATED : October 1, 1985  
INVENTOR(S) : MASAHIRO HARUTA, ET AL.

Page 2 of 2

It is certified that error appears in the above-identified patent and that said Letters Patent is hereby corrected as shown below:

Column 15, line 39, change "stirring" to  
--stirred--.

Column 17, line 7, change "Dry conditions:" to  
--Drying conditions:--.

Column 18, line 35, change "fullcolor" to  
--full-color--.

Signed and Sealed this  
Sixteenth Day of September 1986

[SEAL]

Attest:

DONALD J. QUIGG

Attesting Officer

Commissioner of Patents and Trademarks